

Sept. 13, 1938.

W. F. GLINSMANN

2,129,901

METHOD OF COLORING COAL

Filed June 4, 1935

4 Sheets-Sheet 1



INVENTOR.

WALTER F. GLINSMANN,  
BY *Elis S. Middleton*  
ATTORNEY.

Sept. 13, 1938.

W. F. GLINSMANN

2,129,901

METHOD OF COLORING COAL

Filed June 4, 1935

4 Sheets-Sheet 2



Sept. 13, 1938.

W. F. GLINSMANN

2,129,901

METHOD OF COLORING COAL

Filed June 4, 1935

4 Sheets-Sheet 3



Sept. 13, 1938.

W. F. GLINSMANN

2,129,901

METHOD OF COLORING COAL

Filed June 4, 1935

4 Sheets-Sheet 4



INVENTOR.

WALTER F. GLINSMANN,

BY

Ellis S. Middleton  
ATTORNEY.

## UNITED STATES PATENT OFFICE

2,129,901

## METHOD FOR COLORING COAL

Walter Frank Glinsmann, Jersey City, N. J., assignor to American Cyanamid Company, New York, N. Y., a corporation of Maine

Application June 4, 1935, Serial No. 24,827

12 Claims.

(Cl. 44—6)

The present invention relates to methods for the coloring of coal and the colored coal per se as an article.

It has heretofore been proposed to apply a so-called Prussian Blue to the surface of coal but difficulty has been encountered in commercial practice in securing a uniform and adherent color, that is, one which would stand up under mechanical handling and weathering conditions.

10 The primary object of the present invention is to overcome the above difficulties, to secure colored coal where the color is adherent, cannot be readily rubbed off, is resistant to weathering, is reasonably uniform, and in which coal of various 15 ages of fracture may be so treated as to produce efficient coloring.

To this end, one aspect of the invention contemplates the treatment of freshly fractured coal to produce a colored surface thereon as the age of 20 the fracture has been found to be a material contributing factor in the efficiency of the coloring process. Another aspect of the invention comprises the treatment of old fractured coal so as to produce the equivalent of a freshly fractured 25 surface.

Another aspect contemplates the colored coal as such, as it has been found that one of the main reasons for the high degree of adherence of the color applied as in this invention, is that such 30 color is actually formed integrally on said surface in contradistinction to color formed remote from the coal and then applied thereto. The invention further consists in the detailed methods of treatment, the apparatus for carrying out such 35 methods and the colored coal per se more fully hereinafter shown and described.

In the drawings:

Fig. 1 illustrates a diagrammatic flow sheet in a typical treatment;

40 Fig. 2 shows a diagrammatic lay-out of a preferred form of apparatus carrying out a coal coloring treatment;

Fig. 3 is a transverse section along the line 3—3 of Fig. 2;

Fig. 4 shows a diagrammatic view of a modified form of apparatus;

Fig. 5 is a sectional view along the line 5—5 of Fig. 4;

Fig. 6 is a side elevation showing a diagrammatically modified form of apparatus for the batch treatment of coloring coal;

Fig. 7 is an end view of the device of Fig. 6.

Referring now with more particularity to the embodiment illustrated for the formation of a blue or bronze color on coal and with reference

to the flow sheet of Fig. 1, the freshly fractured coal or coal treated to produce the equivalent of a freshly fractured surface, of which more later, is first washed to remove such objectionable material as dust, slime, mine water and/or excess 5 reducing agent and is then fed into a suitable tumbling or shaking apparatus. In the case of old fractured coal, this tumbling equipment may be such as will mechanically produce the equivalent of a freshly fractured surface, which matter 10 will be more fully discussed hereinafter. In the case of freshly fractured coal, however, this tumbling or shaking apparatus may consist of a chute, trough, or rotary equipment into which the coal is fed and where contact is made with a 15 coloring solution which preferably consists of a freshly mixed solution of an alkali or alkaline earth metal ferricyanide, such as ammonium, sodium, potassium or calcium ferricyanides and a ferric salt solution, such as chlorides, nitrates or 20 sulphates. It is preferable that the tumbling or shaking apparatus, which may be termed a contact apparatus, be provided with means whereby the coal to be treated remains for a requisite 25 length of time in pools of the treating liquid. From this contact apparatus the spent liquid may be drained for re-use if found desirable and the coal so treated and colored is then passed to a 30 washing apparatus and from thence to storage or coal cars for delivery to the consumer. As a 35 matter of fact, the washing subsequent to the coloring treatment may take place remote from the coloring apparatus, either prior to storage, subsequent to storage, prior to loading into the cars or subsequent thereto as circumstances will 40 dictate.

As to the matter of the desirability of freshly fractured surfaces for treatment with the coloring solutions of this invention, it has been found that the greater the interval between fracture and 45 coloring, the less efficient the blue coloring action. This is especially true as to the rate of coloring. This retardation is especially noticeable when the interval approaches an hour. Such coal has a tendency to acquire a bronze effect rather than a 50 blue color. A study of this situation has disclosed that during this period an oxidation of the coal surface or conversion of the atomic carbon to molecular, has taken place to such an extent that the proper reaction between such surface and the coloring solution does not produce an efficiently 55 adherent or uniform blue. This result may be avoided either by treating coal which has been fractured less than that period of time or by treating coal which has been fractured more than that

period with a reducing agent or otherwise, so as to produce on the coal a surface equivalent to one freshly fractured and this discovery is an important element in the present invention. Of course, where a bronze effect is desirable, the treatment may be carried out as above to avoid a blue color and produce a bronze appearance. As a matter of fact, a combination of blue and bronze may thus be secured by suitable compromise of the above circumstances.

Among the materials which have been found to be efficacious in the production of a coal surface equivalent to one freshly fractured may be mentioned reducing agents generally and specifically a solution of sodium bisulphite, sodium sulphite, sulphurous acid, stannous chloride and/or a liquid containing freshly generated hydrogen such as a suspension of finely divided iron in hydrochloric acid. Of these materials, sodium bisulphite is preferred. It is, of course, understood that any metallic salt of these acids may be likewise used in the reducing solution although the sodium salt is preferred from the standpoint of cost. While various concentrations of these reducing agents have been found to be suitable for the purpose, yet a 10% solution has been found to give optimum results. Likewise, the time limit of contact between the reducing agent and the coal may be varied dependent upon the use of the reagent employed and many other circumstances. The time element should be sufficiently long, however, to produce a desirably reduced surface.

It is important that the excess reducing agent be washed from the coal and this is also true of any dust, slime, mine water or other material which might effect the reaction between the coloring solution and the coal be removed prior to the coloring treatment. Of course, if old fractured coal is to be treated with a reducing material, it is desirable that these extraneous materials be washed from such coal prior to the reducing treatment.

The freshly fractured coal or coal having a surface equivalent to that of a fresh fracture may then preferably be fed, as in Fig. 2, from a hopper 1 into a trough 2 suitably supported as at 3 for vibration as by means of an eccentric 4 and suitable connecting mechanism 5. As the coal is fed into the trough 2, a wash spray 6 may be provided for removal either of the dust and slime and other objectionable material which may include the excess reducing agent, the wash water passing through the perforated section 7 of the trough 2 into the wash drain 8 for disposal.

The remainder of the trough 2 beyond the dewatering section is preferably provided with a series of baffles 9 forming depressions therebetween so that the coal in passing through this shaker chute will lie not only in a plurality of layers, but in independent pools of the reagent supplied by means of one or more sprays 10. As above described, it is desirable that this reagent consist either of alkali or alkaline earth ferricyanides freshly mixed with a solution of ferric salts immediately prior to the application to the coal. A suitable mixture has been found to be one consisting of 0.5% ferric chloride and 0.413% calcium ferricyanide freshly mixed and supplied in the proportion of not more than 80 pounds of the mixture to each ton of coal treated.

The shaker chute is provided at the end thereof with a perforated section 11 through which the excess material will drain due to the inclination of the chute into the drainage equipment 12 for

proper disposal. The coal thus treated passes out of the end of the chute 2 into the wash means 13 supplied with a wash spray 14 where any excess coloring solution is removed. The wash water drains from this equipment through the pipe 15 for disposal. This washing step may, of course, be immediately adjacent the end of the coloring equipment, or, on the contrary, may be at some remote point, either prior or subsequent to the storage bins or prior or subsequent to the loading into cars, as found desirable. This later treatment has been found to be particularly desirable as to some types of coal as the longer the treating solution remains in contact with the coal, the better the coloring effect. In the drawings, therefore, the washing equipment is to be taken as a diagrammatic showing as to location.

Another form of suitable equipment is shown in Fig. 4 to consist of a comparatively deep trough 16, all other parts of this equipment being substantially the same as shown in Fig. 2. In this case, however, the fact that the trough is deep as compared to its width increases the depth of the coal layer and the consequent percolation of the reagent increases the coloring efficiency.

In Fig. 6, a batch equipment is illustrated as consisting of a rotary drum 17 provided with the removable manhole or cover 18 into which the material or coal to be treated may be fed through the hopper 19, the two reagents being fed from the tanks 20 and 21 by means of pumps 22 and controlled by means of the valve 23. A perforated pipe 24 arranged axially of the drum provides for the spraying of this mixed reagent onto the coal. Upon charging the drum with a requisite amount of coal and reagent, the valve 23 is closed and the drum rotated through a suitable motor mechanism 25 for a requisite length of time, whereupon the manhole 18 may be removed, the drum rotated until the opening covered by the manhole is over the discharge hopper 26 and the batch discharged. Of course, proper washing and draining apparatus is provided as in the case of Figs. 2 and 4.

It has been found to be unnecessary to confine the batch rotary treatment of Fig. 6 to freshly fractured coal for it has been discovered that old fractured coal, when treated according to this method, acquires a surface equivalent to that of a fresh fracture. This may be due to the tumbling action of one piece of coal on another. At any rate, it is not necessary to especially treat coal fed to this tumbling equipment, although, of course, it may be, if so desired.

In devices of the type shown in Fig. 6, it has been found desirable to use a solution containing 0.5% ferric chloride and 0.413% calcium ferricyanide, freshly mixed, in a proportion of about 46 pounds of the mixed solution per ton of coal treated.

In all of the above treatments, it is desirable that the treating solutions be maintained out of contact with metal and this is particularly true if the ferricyanide and ferric salt solutions are mixed prior to the application to the coal. For this reason, all surfaces coming in contact with such solutions should be non-metallic and be made of such materials as rubber, wood, wood coated with non-metallic containing films such as a synthetic drying oil resin, porcelain or glass, although rubber is preferred.

Coal treated according to the above process and in the above apparatus has been found to have an admirably adherent and uniformly colored surface. This adherence is undoubtedly due to

the fact that the color is not an applied film as has been the case heretofore but, on the contrary, integral with the coal surface, that is, the coal surface itself plays a part in the reaction involving the treating reagent so that the blue color or precipitate actually forms on the surface. This is a new principle of coal coloration.

Mention has been made above that if the time interval between fracture and coloring is prolonged, a bronze effect is produced rather than blue. In some instances, of course, it may be found desirable to produce a bronze color, in which event, either the time interval between fracture and coloring may be deliberately delayed, the reducing treatment may be omitted or the type of apparatus used may be chosen because of its inability to produce the equivalent of a freshly fractured surface such as the tumbling equipment of Fig. 6.

20 In the claims, where the words "freshly fractured surface" are used this is intended to cover any situation where either the coal is freshly fractured so as to make available the substantially atomic carbon of this surface for the reaction, or 25 the equivalent thereof such as is produced either by the use of a reducing agent or by tumbling.

While the invention has been shown and described with reference to particular steps in methods, composition and proportion of ingredients 30 and specific embodiments of apparatus, yet it is to be understood that the invention is not to be restricted thereto but is to be construed broadly and limited only by the scope of the claims.

I claim:

- 35 1. A method of coloring coal which includes subjecting a freshly fractured coal surface to the action of an alkali or alkaline earth ferricyanide and a ferric salt.
2. A method of coloring coal which includes 40 subjecting a freshly fractured coal surface to the action of an alkali or alkaline earth ferricyanide and a ferric salt and subsequently washing said coal.
3. A method of coloring coal which includes

subjecting coal to a treatment to produce a surface thereon equivalent to a freshly fractured surface and subsequently coloring said coal by applying to said surface an alkali or alkaline earth ferricyanide and a ferric salt.

5

4. The method of claim 3 in which the coloring material consists of a mixture of 0.5% ferric chloride solution and 0.413% calcium ferricyanide solution in a proportion of not more than 80 pounds of the mixture to each ton of coal treated.

10

5. The method of claim 3 in which the coloring material consists of a mixture of 0.5% ferric chloride solution and 0.413% calcium ferricyanide solution in the proportion of substantially 46 pounds of the mixture to each ton of coal treated.

15

6. The method of claim 3 in which said treatment comprises washing with a reducing agent.

7. The method of claim 3 in which said treatment comprises washing with a reducing agent as a 10% solution.

20

8. The method of claim 3 in which said treatment comprises washing with a solution containing a material chosen from the group consisting of sodium bisulphite, sodium sulphite, sodium sulphide, sulphurous acid, stannous chloride and 25 freshly generated hydrogen.

9. The method of claim 3 in which said treatment comprises washing with a solution of sodium bisulphite.

10. The method of claim 3 in which said treatment comprises washing with a 10% solution of sodium bisulphite.

30

11. A method of coloring coal which includes agitating and tumbling said coal to produce a surface thereon equivalent to a freshly fractured 35 surface, and subjecting such coal surface to the action of an alkali or alkaline earth ferricyanide and a ferric salt.

12. The method of claim 1 in which the time interval between the coal fracture and the application of the ferricyanide and chloride is not 40 greater than one hour.

WALTER FRANK GLINSMANN.